

# United States Patent [19]

Weaver

[11] 3,912,758

[45] Oct. 14, 1975

[54] **POLYTHIOETHER IMPRESSION MATERIAL**

[75] Inventor: **Benjamin Weaver**, Detroit, Mich.

[73] Assignee: **Sybron Corporation**, Rochester, N.Y.

[22] Filed: **Jan. 28, 1974**

[21] Appl. No.: **437,234**

[52] **U.S. Cl.** ..... 260/33.6 UA; 32/15; 32/17; 106/35; 260/42.37; 260/79; 260/79.1; 260/998.11

[51] **Int. Cl. 2** .... A61K 5/06; C08K 5/01; C08K 5/37

[58] **Field of Search**...260/998.11,79,79.1,33.6 UA; 106/35; 32/15, 17

[56] **References Cited**

UNITED STATES PATENTS

2,558,139 6/1951 Knock et al. .... 32/17  
3,349,047 10/1967 Sheard ..... 260/79.1  
3,736,301 5/1973 Berenbaum et al. .... 260/79.1

3,751,399 8/1973 Lee et al. .... 32/15

**OTHER PUBLICATIONS**

Anderson — Applied Dental Matls., (3rd ed.), (Blackwell Sci. Pub.), (Oxford, England), (1967), pp. 217-219.

Combe — Notes on Dental Matls., (Churchill Livingstone), (London), (1972), pp. 141-142.

*Primary Examiner*—M. J. Welsh

*Assistant Examiner*—H. H. Fletcher

*Attorney, Agent, or Firm*—Theodore B. Roessel; Papan Devnani

[57] **ABSTRACT**

A colorable, pleasant smelling, quick setting, putty-like polythioether polymer material formed by reacting a mercaptan and a diacrylate with the aid of a peroxide catalyst.

**5 Claims, No Drawings**

## POLYTHIOETHER IMPRESSION MATERIAL

## BACKGROUND OF THE INVENTION

The present invention relates to a dental impression material and more particularly to a polythioether impression material. In current practice a two paste system containing polymeric mercaptan, plasticizers, sulfur, lead peroxide and a filler is used by dentists to take impressions of patient's teeth. Such impressions are used by the dentist to make crowns, dentures, or the like. When mixed, usually with a spatula on a paper pad a polymerizable material is formed which the dentist applies to the teeth to produce a custom dental tray. When set, the polymerized material is removed and this custom dental tray used as a mold in making the crown or denture.

The two paste system of the prior art, however, has a relatively long setting time and the fact that the material contains lead may make it somewhat objectionable to the dentist. Furthermore the prior art mixture is an unsightly brown color and has an offensive odor due to the presence of low molecular weight sulfur compounds. For these reasons, putting such a material into the patient's mouth and the taking of a dental impression, often proved to be an unpleasant and traumatic experience. During the time the impression is being taken the patient must keep his mouth steady and immobile and since the curing time of the prior art material is six minutes it is difficult for the patient to do this.

The drawbacks of the prior art are overcome in the present invention by providing an impression material which is lead-free, pleasant smelling, quick setting, and colorable.

## SUMMARY OF THE INVENTION

The present invention is characterized by a dental impression material formed by admixing two paste-like components. A base component comprising a mercaptan terminated polymer and an acrylate monomer, and a catalyst component comprising a metal peroxide and an accelerator. Fillers and plasticizers are added as necessary to improve the mixing characteristics and physical properties.

## OBJECTS OF THE INVENTION

One object of the invention is to provide a polymeric impression material which can be admixed and is aesthetically pleasing.

Another object of the invention is to provide a polythioether dental impression material.

A further object of the present invention is to provide a dimensionally stable dental impression material which has a pleasant odor and which can be given any color.

Yet another object is to provide a dental impression material capable of hardening in approximately  $\frac{1}{2}$  minutes.

## DETAILED DESCRIPTION OF THE INVENTION

The polythioether polymer material of this invention is used for making impression and imprints and serves as a mold from which a similar article could be reproduced. In the uncured stage the polymer has a putty-like consistency. An impression of a shape or a contour is made upon it. Upon curing the polymer hardens and retains the impression. The polymeric material has

non-adhering properties and releases itself easily from the object whose impression is made.

The polythioether impression material of the invention is a polymeric system based on the use of: (1) a mercaptan terminated polymer, more specifically a mercaptan terminated bis(oxyethylene)methane containing disulfide linkage with a small amount of thio groups in the chain, having a molecular weight of 4,000; (2) a di, tri or tetra-acrylate monomer such as hexane diol diacrylate or polyethyleneglycol diacrylate or trimethylolpropane triacrylate; and (3) a peroxide preferably calcium peroxide.

The mercaptan terminated polymer suitable for use in the present invention will in general have a functionality of two or greater and will be of a high molecular weight but still liquid and fluid. It may also contain various amounts of mercapto groups in the chain for cross-linking purposes. The polymers should have molecular weights ranging from 1000-4000 and may contain various percentages of mercapto groups on the molecular chain. The mercapto groups are available for crosslinking the acrylic monomers. Many polymers meeting this description are commercially available. We have found products manufactured by Thiokol Chemical Co. under the trade name LP-2, LP-33, etc. to be particularly useful.

Some examples of di, tri and tetra acrylated monomers and polymers are propylene glycol diacrylate, butylene glycol diacrylate, hexane diol diacrylate, tri methylol propane triacrylate, pentaerythritol tetraacrylate, and polyethylene glycol diacrylate. Properties of the polymerizable system will depend upon the acrylate chosen and the amount used. Functionality of acrylates is chosen to get optimum physical properties in the finished custom dental tray which is used as the mold. With the increase in functionality physical properties such as hardness, and rigidity increases. The excessive amounts lead to shorter pot life, brittleness and higher shrinkage. The molecular weight of acrylate can affect rigidity, elasticity, as well as working time. High molecular weight acrylates such as polyethylene diacrylate produce soft elastic, non-rigid polymers. Hexane diol diacrylate produces polymers having increased hardness and rigidity. Tri acrylates would produce corresponding results depending upon molecular weight. For our purposes we have found that an excess of stoichiometric equivalents is desirable, although less amounts can be used if modifications are desirable in the working characteristics.

Along with the mercaptan terminated polymer and acrylic monomers the use of appropriate fillers is quite necessary to reinforce the set material. Many fillers known in the elastomeric field could be used, such as: calcium carbonate, calcium oxide, magnesium oxide, magnesium sulfate, strontium sulfate, barium sulfate, titanium dioxide, zinc oxide, zinc sulfate, zinc sulfide, zinc chloride, aluminum oxide, silica, antimony oxides, tin oxides, and others. As in most elastomeric applications particle size and surface behavior are important considerations in filler selection.

The plasticizers are used to control the consistency of the hand moldable putty. A number of plasticizers are available for use, depending upon particular properties desired. We have found a low molecular weight liquid styrene polymer to be quite useful as a plasticizer. Suitable plasticizers are those having the viscosity in the range 2000-50000 cps at ambient tempera-

tures. For better results, one within the range of 10000-30000 cps is employed. A suitable plasticizer is TP-680, manufactured by Thiokol Chemical Corp., of Trenton, New Jersey. It has been identified as oligomeric alpha methyl styrene and has the following physical properties:

|                             |             |    |
|-----------------------------|-------------|----|
| Color, Gardner              | 2.5         |    |
| Viscosity at 77°F., poise   | 120-200     |    |
| Volatility 2 hrs. at 311°F. | .55%        | 10 |
| Volatility 4 hrs. at 311°F. | 1.29%       |    |
| Flash point °F. open cup    | 300 maximum |    |
| Fire point °F. open cup     | 350 maximum |    |
| Pour point °F.              | 50          |    |
| Refractive Index            | 1.58        |    |
| Sp. G. at 77°F.             | 1.03        |    |

Metal peroxides are utilized as reactive components. These include zinc peroxide, tin peroxide, antimony peroxide, lead peroxide, manganese peroxide, barium peroxide, strontium peroxide, calcium peroxide, magnesium peroxide, and others. We have also found that hydroperoxides such as cumene hydroperoxide can be useful. For our purposes we have found calcium peroxide to be most desirable because of its good reactivity, good handling, acceptable color and low potential toxicity. Water and amines such as triethylolamine can be further used to accelerate the reaction and improve the physical properties.

These components are formed into two pastes, one containing primarily the base and the other the catalyst. The catalyst component in addition includes the metal peroxide.

A typical base component formed according to the present invention would include:

|                          |        |              |  |
|--------------------------|--------|--------------|--|
| Mercaptan Polymer (LP-2) | 100.00 | parts by wt. |  |
| Hexane Diol Diacrylate   | 6.00   | parts by wt. |  |
| Filler (silica)          | 200.00 | parts by wt. |  |
| Mineral Oil              | 10.00  | parts by wt. |  |
| Perfume                  | trace  | parts by wt. |  |
| Pigment                  | trace  | parts by wt. |  |
| Water                    | 2.00   | parts by wt. |  |

The catalyst component typically would include:

|                    |        |              |  |
|--------------------|--------|--------------|--|
| Plasticizer TP-680 | 70.00  | parts by wt. |  |
| Triethylolamine    | 5.00   | parts by wt. |  |
| CaO <sub>2</sub>   | 100.00 | parts by wt. |  |
| Filler (Silica)    | 190.00 | parts by wt. |  |
| Mineral Oil        | 15.00  | parts by wt. |  |

In order to form a dental impression material according to the present invention, two parts of the base is admixed with one part of the catalyst.



The base and catalyst can be mixed together in the hands and when molded and set, produce a rigid high durometer material having a hardness of 75-80 on a Shore A durometer. The material sets in 1 1/2 minutes and because of absence of low molecular weight sulfur compounds it is void of offensive odor. The ratio of base to catalyst could be varied to control the setting time between 1-5 minutes. An increase in the catalyst amount shortens the time. Another successful formula for these components would include:

|                        |                 |
|------------------------|-----------------|
| <u>Base</u>            |                 |
| Polymercaptan          | 100.00          |
| ZnS                    | 23.00           |
| Trimethylol            | 2.00            |
| propane triacrylate    | parts by weight |
| Hexane diol diacrylate | 2.00            |
| Water                  | 1.50            |
| <u>Catalyst</u>        |                 |
| Calcium peroxide       | 100.00          |
| Magnesium oxide        | 10.00           |
| Zinc oxide             | 100.00          |
| Plasticizer (TP-680)   | 175.00          |
| Mineral oil            | 5.00            |
| Silicone Oil           | 10.00           |

Thus, it should be appreciated that the present invention accomplishes its intended objectives in providing a dental impression material which smells good, is aesthetically pleasant, colorable, easy to handle, and sets in 1 1/2 minutes instead of 6 minutes thereby saving a dentist's time. In addition it is so easy to form a custom tray it saves an additional visit by the patient to the dentist.

Ideally, the polymeric material is most suited as a dental impression material. It could also be used in making reproductions of carvings and sculptures. The impression material is applied on the surface of the sculpture and removed upon hardening. This matrix could then be used to make more copies of the sculpture.

Having described the invention in detail, what is claimed as new is:

1. An impression material formed by polymerization by mixing together two paste like components:

- a. component one comprising;
    - i. an acrylate monomer selected from a group consisting of hexanediol diacrylate, polyethylene glycol diacrylate and trimethylolpropane triacrylate,
    - ii. a mercaptan terminated polymer of molecular weight 1000-4000, having mercaptan groups available for crosslinking with said monomer, and
    - iii. said acrylate monomer making up about 6 parts by weight and said polymer making up about 100 parts by weight of component one;
  - b. component two comprising;
    - i. alpha methyl styrene oligomer as plasticizer,
    - ii. a peroxide catalyst for initiating a reaction between said polymer and monomer of component one;
    - iii. triethylolamine as accelerator for speeding the reaction;
    - iv. said plasticizer making up 70 parts by weight, peroxide catalyst 100 parts by weight and triethylolamine 5 parts by weight of component two; and
  - c. components one and two each further comprising 190-200 parts by weight a filler and 10-15 parts by weight mineral oil.
2. Material of claim 1 wherein the filler is silica.
  3. Material of claim 1 wherein the catalyst is calcium peroxide.
  4. Material of claim 1 wherein said material contains a perfume.
  5. Material of claim 1 wherein said material contains a pigment.

UNITED STATES PATENT OFFICE  
CERTIFICATE OF CORRECTION

Patent No. 3,912,758 Dated October 14, 1975

Inventor(s) Benjamin Weaver

It is certified that error appears in the above-identified patent and that said Letters Patent are hereby corrected as shown below:

Column 1, line 57, change "1/2" to -- 1 1/2 -- ;  
Column 2, line 15, after "two" insert -- (2) --;  
line 27, change "acrylated" to -- acrylate --  
Column 3, line 55, the entire equation should be deleted

Signed and Sealed this  
twentieth Day of January 1976

[SEAL]

Attest:

RUTH C. MASON  
Attesting Officer

C. MARSHALL DANN  
Commissioner of Patents and Trademarks